

Dec. 29, 1953

H. C. COLPITTS

2,664,486

THERMISTOR AND METHOD OF HEAT TREATING IT

Filed June 15, 1951



FIG. 1



FIG. 2



FIG. 3



FIG. 4



FIG. 5

Inventor  
*Harry Colpitts*

By *Robert B. Harmon*

Attorney

## UNITED STATES PATENT OFFICE

2,664,486

THERMISTOR AND METHOD OF  
HEAT-TREATING IT

Harry C. Colpitts, Montreal, Quebec, Canada, assignor to Northern Electric Company, Limited, Montreal, Quebec, Canada, a corporation of Canada

Application June 15, 1951, Serial No. 231,814

5 Claims. (Cl. 201—63)

## 1

This invention relates to thermistors and more particularly to a method of heat treating the thermistor element.

Thermistors, or semi-conductors having a negative resistance-temperature coefficient, have been known for several years. Their value as possible circuit elements has long been recognized. However, one of the reasons for the slow adoption of thermistors into general use has been a difficulty experienced with all semi-conductor elements, that is, the difficulty of obtaining uniform characteristics.

It is the object of this invention to provide a simplified method for the manufacture of thermistors.

It is the further object of this invention to provide a method for producing thermistors of uniform resistance.

It is the further object of this invention to provide means for making an adjustment of the cold resistance after the thermistor element has been assembled in a protective envelope.

It is the further object of this invention to provide a method of reclaiming thermistors whose resistance characteristics have changed due to aging or abnormal use.

An understanding of the invention may be had by reference to the drawings in which:

Fig. 1 illustrates a string of thermistor beads.

Fig. 2 illustrates an individual bead cut from the string.

Fig. 3 shows the thermistor element mounted in a protective envelope.

Fig. 4 shows the resistance distribution of a group of thermistor beads.

Fig. 5 is a chart showing the relation between heating current and bead temperature.

The present art used in the manufacture of bead type thermistors is illustrated in Fig. 1 in which a string of small spheroidal beads 12 of semi-conductor material is formed on a pair of lead wires 11 which support the bead and make electrical contact with it. To do this the pair of lead wires 11, which may be of platinum alloy, are strung on a suitable support. The lead wires used to form the string of Fig. 1 may be about twelve inches in length, four-thousandths of an inch in diameter, and spaced one thirty-second of an inch apart. The semi-conductor material is ground into a paste with a volatile vehicle such as distilled water. Several kinds of semi-conductor materials are known to the art, of which the oxides of cobalt, iron, nickel, zinc, manganese, and uranium have been widely used. A ceramic binder or filler may be included in the paste.

## 2

Small daubs of the paste are placed on the parallel wires at quarter inch intervals. Surface tension pulls the paste into a spheroidal shape.

The beads are dried by evaporating the vehicle, hardened by passing the string of beads shown in Fig. 1 through a small flame, and then sintered by passing through a furnace. Individual beads illustrated in Fig. 2 are then cut from the string and then tested. Beads having the desired resistance characteristic are selected and mounted in an evacuated glass envelope 13, with the lead wires 11 connected to terminal wires 14.

Completed thermistors are required to meet requirements for resistance and delay-time. The delay-time is the time required for the resistance to drop to a given value after the application of a given voltage, and is mainly dependent on the resistance and the size of the bead. If the cold resistance of the bead is within required limits and the size is properly controlled, the thermistor will normally meet delay-time requirements. In giving following information on the changing of resistance of thermistors no mention will be made of delay-time although it must be kept in mind that the delay-time is a function of the resistance.

In the firing process described above, it is necessary to control the furnace temperature, the speed with which the string of beads is pulled through the furnace, the rate of cooling, and the amount of air passing through the furnace. In spite of these controls it is difficult to obtain a uniform resistance characteristic of the bead. The bead and wire assembly is fragile, and is easily subject to mechanical change. Handling of the assembly tends to increase the resistance of the bead. Since it is necessary to handle the bead several times before assembly in the glass envelope is complete, beads which have a desired characteristic after firing may be spoiled or changed during assembly. In addition, differences in individual beads cannot be corrected, since firing a string does not permit of individual adjustment.

Fig. 4 shows a representative distribution of cold resistance values for a group of thermistor beads made according to the present art and tested while in the stage illustrated in Fig. 2. The horizontal axis of Fig. 4 is in thousands of ohms, while the vertical axis is in per cent of the total group for a class interval of 5,000 ohms. Thus the point P indicates that 10 per cent of a representative group of thermistor beads would have a cold resistance in the range 45,000 ohms to

50,000 ohms. From Fig. 4, it is apparent that the yield of thermistors lying within practical resistance limits of  $\pm 25$  per cent is very small. As mentioned above, this is aggravated by further handling of the bead after selection at this stage.

In the method according to this invention, the beads are made in strings as shown in Fig. 1 and passed through the sintering furnace. The individual beads of Fig. 2 are then cut from the string and completely assembled. After assembly, the resistance of the thermistor beads are individually adjusted to the required value by heat treatment. Since the bead is protected by envelope 13, further handling does not alter the characteristics.

According to this invention, the resistance of uranium oxide beads may be adjusted by heat treatment at temperatures from 600 degrees centigrade to 1100 degrees centigrade. This range is well below the initial sintering temperature which may be 1300 degrees centigrade. It has been found that beads which have a resistance below the average of a group may be brought nearer the average by heat treatment at the lower end of the temperature range 600-1100 degrees centigrade. Furthermore, beads which have a resistance above the average of a group may be brought nearer the average by heat treatment at the upper end of the temperature range 600-1100 degrees centigrade.

According to this invention, heating may be accomplished by the passage of a current many times the working current through the bead. Fig. 5 shows a representative relation between surface temperature and heating current for uranium oxide-pyrex beads  $\frac{1}{8}$  inch in diameter. The normal working current for such beads may be a few milliamperes. Quantities expressed in the discussion below are for thermistor beads of this type.

If the bead resistance is above the average of the group, it may be lowered by the momentary application of a heating current of approximately 0.7 ampere. Generally speaking, the larger the heating current (or the higher the temperature), the greater the drop in resistance. However, currents above one ampere yield inconsistent results and may damage the bead permanently. The proper value of heating current may be determined for a group by trial on a few beads. The resistance may not be lowered indefinitely, but behaves as though it were approaching a stable range of values. The beads, or completed thermistors are allowed to cool in air.

If the bead resistance is below the average of the group, it may be increased by successive momentary applications of a heating current of approximately 0.3 ampere. Generally speaking, increasing the number of hot and cold cycles by repeated applications of heating current followed by a cooling period increases the resistance of the bead. The resistance may not be increased indefinitely, but behaves as though it were approaching a stable range of values.

In general, beads which are above the group average for resistance are not affected by heat treating at the lower end of the range 600-1100 degrees centigrade, and beads which are below the group average are not affected by heat treatment at the upper end of the range 600-1100 degrees centigrade.

The heat treating temperatures mentioned above are surface temperatures estimated by means of an optical pyrometer. It will be appreciated that the interior temperature of the bead may be considerably above these values.

Thermistor beads which have changed values due to aging or overloading may be readjusted by the method outlined above.

It is convenient to use a relatively high voltage source of poor regulation to supply the heating current. Thus a 70 volt supply working through a 3500 ohm resistor which may be variable has been found suitable for the heat treatment outlined above.

The behavior of thermistors of initially high resistance is illustrated in the Table I below in which the resistance is expressed in thousands of ohms, and the heating current in amperes:

TABLE I

| Thermistor sample | Initial cold resistance | Cold resistance after heat treating with a current of — |     |     |     |     |
|-------------------|-------------------------|---------------------------------------------------------|-----|-----|-----|-----|
|                   |                         | 0.5                                                     | 0.6 | 0.7 | 0.8 | 1.0 |
| 1.                | 1,500                   | 56                                                      | 53  | 49  | 48  | 43  |
| 2.                | 330                     | 49                                                      | 48  | 46  | 43  | 46  |
| 3.                | 110                     | 53                                                      | 53  | 49  | 49  | 53  |
| 4.                | 93                      | 49                                                      | 49  | 49  | 48  | 43  |
| 5.                | 79                      | 49                                                      | 48  | 48  | 49  | 46  |
| 6.                | 75                      | 47                                                      | 43  | 43  | 37  | 35  |

The behavior of thermistors of initially low resistance is illustrated in Table II below in which the resistance is expressed in thousands of ohms:

| Thermistor sample | Initial cold resistance | Cold resistance after heating with a current of 0.3 ampere and allowing to cool |       |             |
|-------------------|-------------------------|---------------------------------------------------------------------------------|-------|-------------|
|                   |                         | Once                                                                            | Twice | Three times |
| 7.                | 40                      | 43                                                                              | 48    | 52          |
| 8.                | 37                      | 40                                                                              | 43    | 46          |
| 9.                | 35                      | 42                                                                              | 48    | 51          |
| 10.               | 33                      | 43                                                                              | 44    | 56          |
| 11.               | 32                      | 37                                                                              | 42    | 44          |
| 12.               | 30                      | 44                                                                              | 43    | 45          |

What is claimed is:

1. A method of making uranium oxide thermistors with a temperature-resistance characteristic of high accuracy which comprises a pre-forming of the semiconductor element and thereafter heat treating by the momentary dissipation of electric energy in the said element, said energy being very large compared to the normal working capacity of the thermistor.

2. A method of making uranium oxide thermistors with a temperature-resistance characteristic of high accuracy which comprises a pre-forming of the semiconductor element and assembling said element in its protective envelope or holder, and thereafter heat treating the said element by the momentary dissipation of electric energy in it, said energy being very large compared to the normal working capacity of the thermistor.

3. A method of adjusting the resistance of uranium oxide thermistors to obtain a temperature-resistance characteristic of high accuracy whereby the semiconductor element is heat treated by the momentary dissipation in it of electric energy, said energy being very large compared to the normal working capacity of the thermistor.

4. A method of making uranium oxide thermistors with a temperature-resistance characteristic of high accuracy whereby the resistance is adjusted according to the method of claim 3 after the semiconductor element has been as-

sembled into its protective envelope or holder.

5. A method of making thermistors with a temperature-resistance characteristic of high accuracy having a semiconductor element containing uranium oxide in which said element is heat treated in the range 600 to 1100 degrees centigrade by the momentary dissipation in the said element of electric energy.

HARRY C. COLPITTS.

References Cited in the file of this patent

UNITED STATES PATENTS

| Number      | Name     | Date          |
|-------------|----------|---------------|
| 1,906,853   | Hediger  | May 2, 1933   |
| 5 2,197,115 | Randolph | Apr. 16, 1940 |
| 2,271,975   | Hall     | Feb. 3, 1942  |